# EUROPEAN PATENT SPECIFICATION

(11) **EP 0 704 864 B1**
(45) Date of publication and mention of the grant of the patent: **13.11.2002**
(21) Application number: 95115134.9
(22) Date of filing: 26.09.1995
(51) Int. Cl.: H01C 17/02, H01C 17/065, H01C 17/06, H01C 17/30

(54) **Resistor on a ceramic circuit board**
Widerstand auf einer keramischen Platte
Résistance sur circuit céramique

(30) Priority: 28.09.1994 JP 23336594; 09.03.1995 JP 4972395
(43) Date of publication of application: 03.04.1996
(73) Proprietor: SUMITOMO METAL (SMI) ELECTRONICS DEVICES INC., Yamaguchi (JP)
(72) Inventor: Fukaya, Masashi, c/o Sumitomo Metal Ceramics Inc., Mine-shi, Yamaguchi (JP)
(74) Representative: Sandmair, Kurt, Dr. Dr.

(56) References cited:
- DE-A- 2 345 102
- DATABASE WPI Section Ch, Week 8152 Derwent Publications Ltd., London, GB; Class L03, AN 81-95815d & JP-A-56 147 405 (MATSUSHITA ELEC IND KK) , 16 November 1981
- PATENT ABSTRACTS OF JAPAN vol. 013 no. 522 (E-849) ,21 November 1989 & JP-A-01 212402 (TOYOBO CO LTD) 25 August 1989,
- PATENT ABSTRACTS OF JAPAN vol. 013 no. 359 (E-804) ,10 August 1989 & JP-A-01 120003 (NARUMI CHINA CORP) 12 May 1989,
- PATENT ABSTRACTS OF JAPAN vol. 014 no. 467 (E-0989) ,11 October 1990 & JP-A-02 191302 (SHOWA DENKO KK) 27 July 1990,

## Description

### BACKGROUND OF THE INVENTION

### 1. Field of the Invention

The present invention relates to a ceramic circuit board having on its surface an external resistor covered with a glass overcoat. More particularly, the present invention is concerned with a ceramic circuit board having an external resistor which stably maintains an accurate resistance value obtained by trimming.

### 2. Description of the Prior Art

Besides an internal resistor disposed between the layers of a multilayer circuit board, a ceramic circuit board for use in integral circuits is provided with a circuit comprising an external resistor and a conductor pattern printed on the surface of the ceramic circuit board, which contributes toward imparting an advanced function to the ceramic circuit board and reducing the production cost.

In the formation of a resistor on a substrate surface, generally, a conductive substance is added to a glass composition, rendered pasty, printed and sintered into the desired resistor. In the formation of the resistor, occasionally, printing is effected so as to cover the resistor with a glass material and fired to thereby form an overcoat in order to protect the resistor from climatic changes or other environmental influences. The obtained resistor has its resistance value finely adjusted by laser trimming.

Generally, a resistor used in a ceramic circuit board is formed by firing a resistor at 800 to 900°C, printing an overcoat paste comprising a low-melting point glass thereon, and firing at 500 to 600°C. In accordance with the miniaturization of electronic appliances and the higher-density packaging therein, there is the tendency that the ceramic substrate is also provided in multilayer form to comply with higher-density packaging. Further, there is the tendency that use is made of substrate materials which have a low coefficient of thermal expansion in conformity with that of silicon chips to be mounted thereon. Under such circumstance, low-temperature firable substrates are used for circuit boards.

In most of the substrates fired at low temperatures, Ag or Cu is used for the formation of internal conductors in the inner layers. However, the coefficient of thermal expansion of the ceramic substrate is different from that of the internal conductors, and such a difference will generate a strain when the ceramic substrate undergoes repeated firing steps, thereby resulting in an electrical disconnection. In order to obtain a circuit board of high reliability, the number of firing steps should be minimized. Further, for conformity with the thermal expansion of the circuit board, a glass of a low coefficient of thermal expansion should be used in the overcoat as well. Still further, for forming the overcoat by firing at low temperatures, it is preferred that a low-melting point glass be employed in the overcoat. However, the low-melting point glass has a drawback in weather resistance, so that it is required to use a glass having a melting point as high as about the temperature employed for firing the resistor.

It is therefore apparent that a resistor capable of being co-fired with the overcoat is desirably employed in a multilayer structure or a ceramic circuit board of a low thermal expansion coefficient. Such a co-firing leads to a reduction in the production steps and in the plant and equipment investment. However, such a co-firing of the resistor and the overcoat brings about the tendency that the glass of the overcoat confines the bubbles generated from the resistor in the external resistor, thereby causing the bubbles to remain within the fired resistor. When the bubbles remain as confined in the resistor, the problem occurs such that a very close access of a trimming edge to the bubble at the time of laser trimming produces cracks therebetween, resulting in the formation of a resistor lacking in stability in resistance values.

The above situation will be described with reference to the drawings. Fig. 1 is a plan of one form of a conventional external resistor disposed on a substrate of a ceramic circuit board, and Fig. 2 is a sectional view thereof. A wiring material such as a metal paste is printed on a ceramic substrate surface 1, thereby forming a conductor pattern 2 on the surface. Part thereof constitutes an electrode for a resistor 3. The resistor 3 is composed of glass components having a conductive material such as a metal added thereto. The upper part thereof is covered with an overcoat 4 composed of glass materials. The resistor 3 and the overcoat 4 constitute an external resistor 7. The overcoat 4 may either cover each individual resistor 3 a little wider than the same or uniformly cover a wide area of not only a plurality of resistors 3 but also a conductor pattern 2.

The co-firing of the overcoat 4 and the resistor 3 prevents the bubbles 6 generated in the resistor from escaping outside because of the presence of the overcoat 4, thus causing them to remain as confined in the resistor 3. Laser trimming of such an external resistor 7 leads to formation of a trimming channel 5 as shown in the figures which extends through the overcoat 4 and the resistor 3.

Although laser trimming is generally conducted while measuring the resistance value exhibited by the resistor, the presence of the bubbles 6 not only interferes with such precision trimming but also generates microcracks upon access of the trimming channel tip to the bubbles 6. Also, even if there is no occurrence of cracks during trimming, cracks may occur because of the bubbles during the use of the circuit board. Thus, the presence of bubbles in the resistor renders the resistance value exhibited by the resistor inaccurate and renders its resistance value after trimming instable.

### SUMMARY OF THE INVENTION

An object of the present invention is to resolve the above drawbacks of the prior art and specifically to provide a ceramic circuit board having an external resistor obtained by the co-firing of a resistor and an overcoat which does not permit bubbles to remain in the resistor and thereby prevent the cracking during laser trimming or thereafter attributed to the bubbles remaining in the resistor.

The inventors have made intensive studies to find out that the above objects can be attained by using a overcoat glass satisfying specific requirements described in detail hereinafter.

The term "deformation temperature" as used in the present invention refers to the softening temperature of a glass material at which the thermal expansion thereof, which has been increasing linearly as the glass material is heated, comes to stop and then begins to decrease. The method of measuring the thermal expansion itself is stipulated in the Japanese Industrial Standards.

The present invention has been arrived at on the basis of the above finding.

Accordingly, the present invention provides ceramic circuit boards with the following constructions (1) to (5).
(1) A ceramic circuit board having an external resistor prepared by co-firing a resistor and a glass overcoat, the resistor of the external resistor being a low-bubbling resistor, wherein the resistor contains Ag in an amount of 0 to less than 1% by weight and the glass of the resistor has a deformation temperature which is not higher than that of the glass of the overcoat.
(2) A ceramic circuit board having an external resistor prepared by cofiring a resistor and a glass overcoat, the resistor of the external resistor being a low-bubbling resistor, wherein the resistor contains Ag in an amount of at least 1% by weight and the glass of the resistor has such a deformation temperature such that this deformation temperature minus 10 °C is not higher than that of the glass of the overcoat.
(3) The ceramic circuit board as recited in item (1) or (2) above, wherein a glass of the resistor is a CaO-Al₂O₃-SiO₂-B₂O₃ system glass.
(4) The ceramic circuit board as recited in item (1) or (2), wherein a glass of the overcoat comprises 60 to 90% by weight of a CaO-Al₂O₃-SiO₂-Cr₂O₃-B₂O₃ system glass and 10 to 40% by weight of alumina, the glass having a deformation temperature of 720 to 740°C.

### BRIEF DESCRIPTION OF THE DRAWINGS

Fig. 1 is a view illustrating a conventional external resistor.

Fig. 2 is a sectional view of the resistor of Fig. 1.

Fig. 3-10 show the change in resistivity versus the difference in deformation temperature between the glass used in a resistor and the glass used in an overcoat.

Fig. 11-18 show the change in resistivity versus the number of bubbles remaining in resistors.

### DETAILED DESCRIPTION OF THE PREFERRED EMBODIMENTS

According to the present invention, the deformation temperature of the glass of the resistor of the external resistor is rendered equal to or lower than that of the glass of the overcoat to provide an excellent low-bubbling resistor, even if the glass overcoat and the resistor are co-fired. This is because the glass of the resistor has a deformation temperature equal to or lower than that of the overcoat by adding 0 to less than 1% of an Ag component to the resistor, so that the sintering of the resistor is accelerated to thereby allow the generated bubbles to escape to the side of the glass overcoat, or because, in addition to an electric resistance component such as RuO₂-based or Bi₂Ru₂O₇-based component, Ag is positively added in an amount of at least 1% to the resistor, so that Ag combines with the resistor materials to thereby promote sintering with the same result that the sintering of the resistor is accelerated to thereby allow generated bubbles to escape from the side of the glass overcoat.

The ceramic circuit board of the present invention may have any monolayer or multilayer construction as long as a ceramic is used as an insulator. A multilayer ceramic circuit board can be produced by, for example, the green sheet lamination process or the printing lamination process. A circuit may be provided only on one side of the substrate or on both sides thereof.

The ceramic material composing the ceramic substrate for use in the present invention is not particularly limited, examples thereof including alumina (Al₂O₃), aluminum nitride (AlN), silicon carbide (SiC) and various ceramics composed mainly thereof. A low-temperature firing ceramic can be used which is a mixture of alumina powder with glass powder. The conductor material used in the inner layers is varied depending on the substrate material. When the substrate material is alumina or aluminum nitride, use is made of a high-melting point metal such as molybdenum or tungsten. When the substrate material can be fired at relatively low temperatures, use is made of a metal such as gold, silver, silver-palladium alloy, copper or nickel.

A ceramic circuit board in which W or Mo is used as a wiring conductor on a substrate of alumina, aluminum nitride or the like and of which the co-firing is conducted in a reducing atmosphere for preventing the oxidation of the conductor is known as an example of the co-fired ceramic circuit boards produced by co-firing a ceramic green sheet and a wiring conductor paste. However, this encounters the problem that conductor oxidation cannot be avoided in the formation of RuO₂-type or Bi₂Ru₂O₇-type resistors of high reliability which must be fired in the air.

On the other hand, a low-temperature firable multilayer ceramic circuit board in which use is made of an Ag-based conductor which has a low circuit resistance and can be fired in the air, such as Ag, Ag-Pd, Ag-Pt or Ag-Pd-Pt, and in which a ceramic material capable of being fired at temperatures not higher than the melting point of the above conductor material (900 to 1200°C) is used as an insulator has been developed, which is especially preferred as the ceramic circuit board of the present invention. Generally, a ceramic board to be fired at about 1200°C or below is called a "low-temperature firable ceramic board", in which, for example, an Ag-based, Au-based or Cu-based conductor is used as conductors on inner layers and surface layers.

A ceramic material which can be fired at temperatures lower than the melting point of, for example, inserted Ag conductor material is preferably employed as the low-temperature firable ceramic insulator material. When use is made of an Ag conductor or an Ag alloy conductor in which the contents of Pd and Pt are low, because the melting point of such a metal formed in multiple layers is as low as about 900 to 1200°C, it is necessary to employ a material which can be fired at 800 to 1100°C. Representative examples of such materials include a mixture of the powder of a glass such as a borosilicate glass or a glass further containing some oxides (e.g., MgO, CaO, Al₂O₃, PbO, K₂O, Na₂O, ZnO, Li₂O, etc.) with the powder of a ceramic such as alumina or quartz, and a crystallizable glass powder which undergoes cordierite or α-spodumene crystallization.

The above material can be used not only in the monolayer form mentioned above but also in the multilayer form. The multilayer substrate can be produced according to the green sheet lamination process in which a plurality of green sheets are employed. For example, a powdery ceramic insulator material is mixed with additives, such as a solvent, resin, etc., and molded according to the doctor blade method into green sheets of about 0.1 to 0.5 mm in thickness. A paste of a conductor material such as Ag, Ag-Pd, Ag-Pt or Ag-Pd-Pt is screen printed on one of the green sheets to thereby give a desired wiring pattern. Through holes each of about 0.1 to 2.0 mm in diameter are formed in the green sheet by means of blanking dies or a punching machine so as to enable connection to another conductor layer. Also, wiring via holes are formed and filled with an Ag conductor material. In the same manner, wiring patterns are printed on other green sheets as many as required for forming the desired circuit. These green sheets are accurately laminated one upon another with the use of tooling holes respectively formed in the green sheets and unified by thermocompression bonding effected at 80 to 150°C under 10 to 250 kg/cm².

When the circuit includes an inner resistor or resistors, an RuO₂ system, or Bi₂Ru₂O₇ system resistor is formed which is fired in the air. In that case, it is printed together with terminals therefor on the green sheet for forming an inner layer.

The obtained structure is co-fired in the air, thereby providing a ceramic multilayer board with built-in conductors.

The present invention has been described with the low-temperature firable ceramic as an example. Although it is a preferred embodiment of the present invention, the present invention is not limited thereto.

The resistors used in the present invention include those composed of a RuO₂-based or Bi₂Ru₂O₇-based electric resistance component and a glass component and, generally, is printed in the form of a paste on a ceramic substrate surface according to the thick-film process. Further, an overcoat composition comprising, for example, a CaO-Al₂O₃-SiO₂-Cr₂O₃-B₂O₃ system glass is printed on the printed resistor, generally by the thick film process. In the present invention, the resistor and glass overcoat are co-fired. The firing is conducted in the air.

The present invention will now be described in greater detail with reference to the following Examples and Comparative Examples.

### EXAMPLES

A ceramic circuit board was prepared with the use of a low-temperature firable ceramic prepared according to the following procedure. 60% by weight of glass powder composed of, in weight percentages, 27% of CaO, 5% of Al₂O₃, 59% of SiO₂ and 9% of B₂O₃ was mixed with 40% by weight of Al₂O₃ powder having an average particle size of 1.0 µm to prepare a powder component.

The above powder component was mixed with, in weight percentage, 10% of acrylic resin, 30% of toluene, 10% of isopropanol and 5% of dibutyl phthalate with respect to 100% by weight of the powder component in a ball mill and formed into a green sheet of 0.4 mm in thickness according to the doctor blade process. This green sheet was punched at given positions by means of dies and an Ag paste was screen printed to fill the holes therewith. The sheet was dried and the Ag paste was screen printed on the sheet to thereby form a wiring pattern. In the same manner, other green sheets having printed wiring patterns were prepared. A given number of obtained sheets were laminated one upon another and caused to undergo thermocompression bonding. The resultant laminate was fired by holding it at 900°C for 20 min. Thus, a ceramic circuit substrate was obtained.

Each of the resistor compositions having the chemical compositions specified in Table 1 was printed on the ceramic substrate so as to form a resistor of 1 mm in width and 2 mm in length. The overcoat was formed by printing on the above resistor, each overcoat composition including each of the glass compositions A to H of Table 2 having respective deformation temperatures indicated in the table, with which Al₂O₃ powder was mixed.

With respect to each of various combinations of these resistors with glass overcoats, a simultaneous firing was performed in the air at 890°C for 10 min.

Each resultant resistor was laser-trimmed so that the resistivity was increased to twice its initial resistivity. The initial resistivities are shown in Table 3.

The RuO₂ content in the resistor material indicated in Table 1 means the weight % based on the total weight of the resistor including Ag and glass components. Likewise, the Ag content means the weight % based on the total weight of the resistor including glass components, RuO₂ and Ag.. The load test indicated in Table 4 means the maximum of the percentage of change in resistivity with respect to the laser-trimmed resistivity, observed after 1000-hrs continuous application of 1/32 W load.

Figs. 3-10 show the relationship between the percentage of the change in resistivity and the difference in deformation temperature between the glasses used in the resistors and the overcoats. The difference was obtained by subtracting the deformation temperature of a glass used in a resistor from the deformation temperature of a glass used in an overcoat (i.e., the deformation temperature of a glass used in an overcoat minus the deformation temperature of a glass used in a resistor). In the figures, for resistors without the addition of Ag, the test results are indicated by the solid circle symbol (●) and region A (hatched with thin lines) is an acceptable range. While, for resistors with the addition of Ag, the test results are indicated by the open circle symbol (○) and region B (hatched with thick lines) is an acceptable range. In Fig. 8, the change in resistivity was relatively large because the yield point of the glass used in the overcoat was high and sufficient sintering was not performed at the firing temperature of 890°C.

With respect to each of the various combinations of resistors 1 to 24 with glass overcoats A to H, Table 4 gives the load test results in terms of the maximum of the percentages of change of resistivity. Table 5 lists the number of bubbles of at least 5 µm in diameter contained in a section of 300 µm x 15 µm which was measured by an electron microscope observation of a section of each resistor.

Figs. 11-18 show the relationship between the percentage of the change in resistivity and the number of bubbles remaining in the resistor.

With respect to various combinations of resistors 1 to 24 with glass overcoats A to H as listed in Tables 4 and 5, the examples of the present invention in which the deformation temperature of the glass of the resistor is not higher than that of the overcoat glass are combinations of glass overcoat A with resistors 1 to 14, glass overcoat B with resistors 3 to 8, 13 and 14, glass overcoat C with resistors 1 to 14, glass overcoat D with resistors 3 to 8 and 11 to 14, glass overcoat E with resistors 3 to 8 and 11 to 14, glass overcoat F with resistors 1 to 14, 16, 18, 21 and 23, glass overcoat G with resistors 1 to 14, and glass overcoat H with resistors 5 to 8, 13 and 14. The examples exerting the same effects as at the deformation temperature of the glass of the resistor minus 10°C, by virtue of the addition of at least 1.0% of Ag, are combinations of glass overcoat A with resistors 15, 17, 19, 20, 22 and 24, glass overcoat B with resistors 15, 17, 19, 20, 22 and 24, glass overcoat C with resistors 15, 17, 19, 20, 22 and 24, glass overcoat D with resistors 15, 17, 19, 20, 22 and 24, glass overcoat E with resistors 15, 17, 19, 20, 22 and 24, glass overcoat F with resistors 15, 17, 19, 20, 22 and 24, glass overcoat G with resistors 15, 17, 19, 20, 22 and 24, and glass overcoat H with resistors 17 and 24. The other combinations are comparative examples to the present invention.

It is apparent from Tables 4 and 5 that, when use is made of, for example, glass overcoat G, as demonstrated by the combinations with resistors 1 to 14, rendering the deformation temperature of the glass of the resistor equal to or lower than the deformation temperature of the overcoat glass causes the sintering of the resistor to precede that of the overcoat glass, so that the number of bubbles is markedly small with excellent load test results so that the rate of change is not greater than 1%. Generally, the reliability of the thick-film resistor is evaluated on whether the change in acceleration test is within ±1% as a rule of thumb. Further, for example, comparison of the combinations with resistors 15, 17, 19, 20, 22 and 24 to the combinations with resistors 16, 18, 21 and 23 as comparative examples shows that the addition of Ag promotes the sintering of the resistor, so that the number of generated bubbles is nil or extremely small, thereby ensuring excellent results in the load test.

It is apparent that the addition of Ag in an amount of at least 1.0% exerts the same effect as a temperature fall of 10°C from the deformation temperature in respect of the promotion of the sintering of the resistor. However, the addition of Ag in an amount greater than 10% causes Ag particles to precipitate, thereby lowering the resistance value.

As apparent from the foregoing, the present invention provides a ceramic circuit board having an external resistor formed by co-firing a resistor and an overcoat, prevents the cracking of the resistor at the time of trimming and thereafter, and realizes the provision of a resistance performance that ensures excellent weather resistance and stability.

## Claims

1. A ceramic circuit board having an external resistor prepared by co-firing a resistor and a glass overcoat, the resistor of the external resistor being a low-bubbling resistor,
wherein the resistor contains Ag in an amount of 0 to less than 1% by weight and the glass of the resistor has a deformation temperature which is not higher than that of the glass of the overcoat.

2. A ceramic circuit board having an external resistor prepared by co-firing a resistor and a glass overcoat, the resistor of the external resistor being a low-bubbling resistor,
wherein the resistor contains Ag in an amount of at least 1% by weight and the glass of the resistor has such a deformation temperature that the deformation temperature minus 10 °C is not higher than that of the glass of the overcoat.

3. The ceramic circuit board as recited in Claim 1 or 2, wherein the glass of the resistor is CaO-Al₂O₃-SiO₂-B₂O₃ system glass.

4. The ceramic circuit board as recited in Claim 1 or 2, wherein a glass of the overcoat comprises 60 to 90% by weight of CaO-Al₂O₃-SiO₂-Cr₂O₃-B₂O₃ system glass and 10 to 40% by weight of alumina, the glass having a deformation temperature of 720 to 740°C.

## Patentansprüche

1. Keramikschaltplatte mit einem externen Widerstand, hergestellt durch gemeinsames Brennen eines Widerstands und einer Glasdeckschicht, wobei der Widerstand des extemen Widerstandes ein Widerstand mit wenig Blasen ist,
wobei der Widerstand Ag in einer Menge von 0 bis weniger als 1 Gew.-% enthält und das Glas des Widerstands eine Verformungstemperatur hat, die nicht höher ist als die des Glases der Deckschicht.

2. Keramikschaltplatte mit einem externen Widerstand, hergestellt durch gemeinsames Brennen eines Widerstands und einer Glasdeckschicht, wobei der Widerstand des externen Widerstandes ein Widerstand mit wenig Blasen ist,
wobei der Widerstand Ag in einer Menge von mindestens 1 Gew.-% enthält und das Glas des Widerstands eine solche Verformungstemperatur hat, dass die Verformungstemperatur minus 10°C nicht höher ist als die des Glases der Deckschicht.

3. Keramikschaltplatte nach Anspruch 1 oder 2, in der das Glas des Widerstandes Glas des Systems CaO-Al₂O₃-SiO₂-B₂O₃ ist.

4. Keramikschaltplatte nach Anspruch 1 oder 2, in der das Glas der Deckschicht 60 bis 90 Gew.-% Glas des Systems CaO-Al₂O₃-SiO₂-B₂O₃ und 10 bis 40 Gew.-% Aluminiumoxid umfasst, wobei das Glas eine Verformungstemperatur von 720 bis 740°C hat.

## Revendications

1. Carte imprimée en céramique ayant une résistance externe préparée par cuisson en commun d'une résistance et d'une couche de finition de verre, la résistance de la résistance externe étant une résistance à faible bullage,
dans laquelle la résistance contient Ag selon une quantité de 0 à moins de 1 % en poids et le verre de la résistance a une température de déformation qui n'est pas supérieure à celle du verre de la couche de finition.

2. Carte imprimée en céramique ayant une résistance externe préparée par cuisson en commun d'une résistance et d'une couche de finition de verre, la résistance de la résistance externe étant une résistance à faible bullage,
dans laquelle la résistance contient Ag selon une quantité d'au moins 1 % en poids et le verre de la résistance a une température de déformation telle que la température de déformation moins 10°C n'est pas supérieure à celle du verre de la couche de finition.

3. Carte imprimée en céramique selon la revendication 1 ou 2, dans laquelle le verre de la résistance est un verre à système CaO-Al₂O₃-SiO₂-B₂O₃.

4. Carte imprimée en céramique selon la revendication 1 ou 2, dans laquelle un verre de la couche de finition comporte 60 à 90 % en poids d'un verre à système CaO-Al₂O₃-SiO₂-Cr₂O₃-B₂O₃ et 10 à 40 % en poids d'alumine, le verre ayant une température de déformation de 720 à 740°C.
